

May 29, 1928.

1,671,491

H. SCOTT

BIMETALLIC ELEMENT

Filed Dec. 27, 1926



WITNESSES:

E. A. McCloskey.  
G. B. Goff

INVENTOR

Howard Scott.  
BY  
Wesley S. Carr  
ATTORNEY

## UNITED STATES PATENT OFFICE.

HOWARD SCOTT, OF WILKINSBURG, PENNSYLVANIA, ASSIGNOR TO WESTINGHOUSE ELECTRIC & MANUFACTURING COMPANY, A CORPORATION OF PENNSYLVANIA.

## BIMETALLIC ELEMENT.

Application filed December 27, 1926. Serial No. 157,322.

My invention relates to thermostatic devices and particularly to bimetallic elements therefor.

An object of my invention is to provide a bimetallic element for a thermostatic device, that shall deflect uniformly over a wide range of temperatures.

Another object of my invention is to provide a bimetallic element for a thermostatic device in which the cooperating elements thereof have substantially equal temperature coefficients of expansion at relatively low temperatures but have widely different temperature coefficients of expansion at relatively high temperatures.

Another object of my invention is to provide a bimetallic element that shall have reversible deflection characteristics.

A further object of my invention is to provide a bimetallic element that shall have uniform deflection over a range of 200° C. and

A still further object of my invention is to provide a bimetallic element that shall have elastic deflection up to 500° C.

In practicing my invention I provide a bimetallic element for thermostatic devices which comprises two cooperating alloys suitably joined together. One of the alloys contains iron and manganese, the manganese content not exceeding 30° of the alloy aggregate. The other alloy may be one having low expansion characteristics similar to that of a nickel-iron alloy.

It is well known that pure iron, upon being heated, passes through a transformation point at approximately 900° C. and, upon still further heating, passes through a second transformation point at substantially 40 1400° C. The structure of the iron below 900° C. is commonly known as Alpha crystalline structure. Between 900° C. and 1400° C. the crystalline structure of pure iron is known as Austenite or Gamma iron and above 1400° C. the crystalline structure changes to that known as Delta iron.

Upon being heated, pure iron expands uniformly up to 900° C. and has a temperature coefficient of expansion of approximately 50  $12 \times 10^{-6}$  cm. per degree C. and between 900° C. and 1400° C., or between its first and second transformation points, it expands uniformly but at a much higher rate, the coefficient of expansion being approximately

$20 \times 10^{-6}$  cm. per degree C. Above 1400° C. 55 pure iron expands at a lower rate than iron having an austenitic structure.

I have found that an alloy containing relatively pure iron and a substantial quantity of manganese possesses substantially the same expansion characteristics upon heating as iron having an austenitic crystalline structure, over a temperature range from +150° C. to +500° C. This alloy is reversible in its thermal characteristics over this temperature range; that is, it follows the same expansion curve on heating as on cooling.

Between 100° C. and about 125° C., I have found that the manganese iron alloy has a temperature coefficient of expansion that 70 does not differ appreciably from that of a nickel-iron alloy, but above 125° C. the manganese-iron alloy has a much higher temperature coefficient of expansion. The manganese-iron alloy, when joined with an alloy 75 having a relatively low coefficient of expansion to form a bimetallic element, is very useful in thermostatic devices as will hereinafter be set forth.

In the single sheet of drawings, the temperature expansion curves of two alloys and of a bimetallic element comprising these alloys are illustrated.

In the drawings, the vertical scale represents expansion in thousandths per unit 85 length and the horizontal scale represents temperature in degrees C. The temperature expansion curve illustrated by numeral 11 represents the expansion characteristic of an alloy containing manganese, iron and a 90 minor percentage of carbon. The curve designated by numeral 12 represents the thermal expansion characteristics of a nickel-iron alloy that forms a bimetallic element with the alloy represented by the 95 curve 11. The curve 13, illustrated by a broken line, represents the difference in expansion between the alloys of curves 11 and 12, to which the deflection of a bimetallic element composed of these alloys is directly 100 proportional under appropriate conditions.

The alloy represented by curve 11 has a very high temperature coefficient of expansion between 100° C. and 500° C. Between 100° C. and -150° C., the expansion coefficient decreases and approximates the temperature coefficient of expansion of the alloy represented by the curve 12. It is to be

- noted that, between  $-150^{\circ}$  C. and  $+100^{\circ}$  C., the difference in the ordinates of the curves 11 and 12 is substantially zero, as indicated by the curve 13. From  $100^{\circ}$  C. to  $400^{\circ}$  C., the differences in expansion of the alloys 11 and 12 is very marked and is of a uniform character. The bimetallic element represented by the curve 13 retains an elastic expansion at a temperature of about  $500^{\circ}$  C.
- 10 The thermal characteristic of the alloy represented by the curve 11 may be varied by changing the manganese content between the limits of substantially 15% and 30% and by moderate additions of other alloying elements. The alloy represented by the curve 12 may be a nickel-iron alloy having any desired temperature coefficient of expansion that is suitable for use with the manganese-iron alloy.
- 15 20 I have found that a bimetallic element comprising a 45% nickel-iron alloy and a ferrous alloy containing substantially 23% manganese and .1% carbon is very sensitive to changes in temperature between the temperatures of substantially  $150^{\circ}$  C. to  $400^{\circ}$  C. Between  $150^{\circ}$  C. and  $-150^{\circ}$  C., this bimetallic element has, for practical purposes, zero expansion. Therefore, it is not subjected to high mechanical stresses in this 25 30 temperature range.
- 35 It is to be understood that the nickel content of the alloy represented by curve 12 may be varied in accordance with the amount of manganese or other additional alloying elements in the alloy represented by curve 11 in order that a bimetallic element may be obtained for thermostatic devices that is operable over a relatively wide range of temperatures in which it is to be responsive, and that is substantially non-responsive to temperatures which are not included within the desired operating range.
- 40 45 While I have designated the curve 12 as being representative of the temperature expansion characteristic of a ferrous alloy containing nickel, I do not wish to be limited to use of this alloy as other alloys having a low temperature coefficient of expansion may be employed. However, the nickel 50 content of the alloy mentioned above may in some instances be materially less than 45% of the alloy aggregate.
- 55 60 Various modifications may be made in the device embodying my invention without departing from the spirit and scope thereof. I desire, therefore, that only such limitations shall be placed thereon as are imposed by the prior art and the appended claims.
- I claim as my invention:
- 65 70 1. A thermostatic element comprising two metals having different temperature coefficients of expansion, one of said elements being an alloy of manganese and iron, and the other of said elements being a ferrous
- 75 80 85 90 95 100 105 110 115 120 125 alloy containing a substantial quantity of nickel.
2. A thermostatic element comprising two metals having different temperature coefficients of expansion, one of said elements being a ferrous alloy containing carbon and manganese, said manganese content being predominant, and the other of said elements being an alloy containing a substantial quantity of nickel.
3. A thermostatic element comprising two metals having different coefficients of expansion, one of said elements being a ferrous alloy containing substantial amounts of nickel and the other of said elements being a ferrous alloy containing a substantial quantity of manganese.
4. A thermostatic element comprising two metals having different coefficients of expansion, one of said elements being a ferrous alloy containing substantial amounts of nickel and the other of said elements being an alloy containing carbon, and manganese, said manganese content being predominant.
5. A thermostatic element comprising two metallic elements having different coefficients of expansion, one of said elements being a ferrous alloy containing not less than 15% of manganese, and the other of said elements being a nickel-iron alloy.
6. A thermostatic element comprising two metallic elements having different coefficients of expansion, one of said elements containing not more than 30% manganese, and the other of said elements being a ferrous alloy containing a substantial quantity of nickel.
7. A thermostatic element comprising two metallic elements having different coefficients of expansion, one of said elements containing from 15% to 30% of manganese, and the other of said elements being an alloy containing a substantial quantity of nickel.
8. A thermostatic element comprising two metallic elements having different coefficients of expansion, one of said elements being an alloy containing manganese and carbon, the manganese content being not less than 15%, and the other of said elements being an alloy containing a substantial quantity of nickel.
9. A thermostatic element comprising two metals having different temperature coefficients of expansion, one of said metals being a ferrous alloy containing substantially 45% nickel, and the other metal being an alloy containing substantially 23% of manganese, 0.1% of carbon, and iron.
- In testimony whereof, I have hereunto subscribed my name this 21st day of December, 1926.

HOWARD SCOTT.